

## UNITED STATES PATENT OFFICE

2,025,486

## IMPREGNATING MATERIAL

Benjamin J. Victor, Oak Park, Ill., assignor to  
 Victor Manufacturing & Gasket Company, Chi-  
 cago, Ill., a corporation of Illinois

No Drawing. Application July 18, 1933,  
 Serial No. 680,992

3 Claims. (Cl. 91—68)

This invention relates to an improved impregnating material, and has for one of its principal objects the provision of an impregnator for textile material and the like, which shall render the 5 same waterproof and also proof against the action of various other liquids, particularly petroleum products.

One of the important objects of this invention is the provision of a textile impregnator which, 10 in addition to rendering a textile material or the like proof against attack by various liquids, shall at the same time leave the same in condition for suitable working and for the ordinary applications to which said textile material has previously 15 been put.

A further important object of the invention is to provide an impregnating compound for certain textile materials or the like, as, for example, asbestos, which impregnator, in addition to rendering the asbestos waterproof, shall also make the 20 same proof against the attacks of liquid hydrocarbons, and in conjunction with the fireproof properties of the asbestos itself, shall also aid in preventing decomposition under extreme heat.

Another and still further important object of the invention resides in the provision of a compound particularly adapted for use in making gaskets for internal combustion engines, which 25 gaskets include an asbestos filler or sheet, and which asbestos, when impregnated with the material of this invention, shall be rendered waterproof and also proof against the action of gasoline or the like, in addition to being made extremely tough and compact while at the same 30 time retaining its desirable resilient qualities.

Other and further important objects of the invention will be apparent from the disclosures in the following specification.

The invention, in a preferred form, is herein- 40 after more fully described.

The improved composition of this invention may be prepared, and the textile material or asbestos may be impregnated to render the same water and gasoline proof in any one of a number 45 of related methods and with certain variations in the materials used.

One of the preferred embodiments of the invention is the incorporation of aluminum stearate into the textile material, asbestos or the like for impregnating purposes to render the same proof against the action of water and other materials.

In order to conveniently employ the aluminum stearate, it is dissolved in a suitable solvent such 55 as, for example, carbon tetrachloride or a similar

material. Mixtures of carbon tetrachloride with other liquids or solvents, as, for example, benzol, may also be employed. The solution is usually facilitated by the addition of heat, and it has been found that the use of a temperature of around 5 140° F. is quite satisfactory when carbon tetrachloride alone is employed for the dissolving of the aluminum stearate.

The proportions used can be varied considerably, depending upon the desired viscosity of the 10 resulting solution, one part by weight or volume of aluminum stearate to five parts by weight or volume of carbon tetrachloride having been found to be quite feasible. Care must be taken in dissolving the stearate in the liquid in order to 15 prevent air bubbles from forming.

After complete solution has taken place, the material can be reduced, if desired, with a suitable thinner so as to provide for a more ready impregnation. This thinner may comprise an 20 addition of the original or a different solvent. The solution can thereby be brought to any desired point of viscosity, so that the same will readily penetrate a sheet of textile material or a sheet of asbestos fibers, hemp or jute fibers, or any 25 other textile or similar material which it is desired to impregnate by the improved composition of this invention.

To improve the solution so as to render the impregnable material more flexible, 1 to 5% of a 30 free fatty acid material may be added. This is thoroughly mixed, and it has been found that asbestos or similar material will thus become impregnated quite thoroughly and to such an extent that the same is rendered completely waterproof and also proof against the action of liquid hydrocarbons such as gasoline, which is quite desirable when the asbestos is used in the manufacture of gaskets for internal combustion engines.

The material can then be dried, preferably 35 without the application of heat and under merely a forced draft of air, the omission of heat being particularly important when the free fatty acid has been added to the solution.

The carbon tetrachloride vapors carried off in the drying process may be reclaimed.

Another impregnating compound is prepared by partially decomposing the aluminum stearate 50 or similar material, this being preferably done at a temperature of around 400° F. and over a sulphuric acid bath, the vapors of the acid acting upon the impurities formed by the aluminum stearate while decomposing. This process also 55

acts in a great degree to prevent the possibilities of undesirable foaming and bubbling over.

After the aluminum stearate has been totally dissolved, it assumes a gummy consistency, and if allowed to cool to room temperature, will resemble to a great degree and will take on many of the characteristics of an artificial resin, and in this condition, is completely soluble in benzol or a similar solvent.

- 10 In order to reduce the dangers inherent to the use of the inflammable benzol, a considerable amount of carbon tetrachloride or some other noninflammable solvent may be added to the benzol, and the decomposed aluminum stearate, when taken up in solution, may then be further thinned and used for impregnating purposes in substantially the same manner as the dissolved powdered aluminum stearate described above. After the desired saturation of the asbestos or other textile material has been accomplished, the benzol, carbon tetrachloride or other solvents may be accordingly reclaimed.
- 15
- 20

The use of the above process results in an impregnating material which, when applied to asbestos or the like, thoroughly penetrates the fibers thereof, and after the solvent has been evaporated off, the aluminum stearate has become so thoroughly incorporated into the fabric or fibers that an absolutely waterproof material results, and one which is also peculiarly resistant to the actions of other liquids, notably hydrocarbons. It is this property which renders the impregnated asbestos particularly valuable for gasket purposes. The material is accordingly toughened and rendered considerably more flexible, and the tendency of the fibers to separate is practically eliminated, while at the same time the desired flexibility and workability is retained.

Another embodiment of the invention is the use of turpentine oil as a solvent for the aluminum stearate. Six parts of turpentine oil will dissolve one part of aluminum stearate with gentle heating, and after cooling, the solution will set to a jell which can be diluted by adding more solvent. An addition of ethyl alcohol to the latter will impart considerably greater liquidity.

The turpentine oil may also be used to further dissolve the jells obtained with carbon tetrachloride and benzol. The use of turpentine with the carbon tetrachloride will probably be preferable on account of the lessened fire hazard.

Another modification of the invention is the actual forming of an aluminum stearate or an aluminum soap within the fiber through the inter-action of soap and aluminum sulphate. This also produces a very good and satisfactory gasket material. Iron may also be substituted for aluminum and iron oleate for stearate.

The latter is preferably pre-treated with a two per cent copperas solution, and after drying, saturated with a casein glue solution containing two per cent ammonium oleate, and again dipped into

the copperas solution, thereby forming two films of a metallic oleate which envelop the casein glue layer on both sides.

While aluminum stearate is the preferred saturant, other metallic salts of fatty acids may be employed, such as oleates or combinations of stearates and oleates may be used. This particular saturant is sufficiently clear and can be made of a desired viscosity so as to penetrate and act as a proofing material for various textiles and fibrous materials other than asbestos, such as hemp and jute fibers. By saturating hemp and jute fibers, a new vegetable fiber packing for shafts is available which has both gasoline and waterproof qualities. One of the main objections to a rope vegetable fiber packing and the saturants heretofore employed therewith is that a corrosion or caustic action takes place when used between two magnesium metals. The use of the saturant of this invention provides a saponification action, particularly when a slight excess of a free fatty acid is used, and this produces a water insoluble soap whereby an ideal packing results, particularly adapted for use with water pump shafts of automobile engines and the like.

After treatment, that is, when the volatile portions have been driven off, the packing is absolutely moisture free, and neither is there any free acid or alkali present, and accordingly, no chemical or physical changes can take place in the saturant, while at the same time it is quite impervious to heat, remaining inert at least up to a temperature of 250° F.

I am aware that many changes may be made and numerous details of the method varied throughout a wide range without departing from the principles of this invention, and I, therefore, do not purpose limiting the patent granted hereon otherwise than as necessitated by the prior art.

I claim as my invention:

1. An impregnating material for gaskets comprising aluminum stearate partially decomposed to a gummy consistency in solution with benzol and carbon tetrachloride with a suitable thinner.
2. A method of liquid proofing a gasket, including the preliminary partial decomposition of a metallic fatty acid salt to a gummy consistency, the dissolving of the resinous residue in a suitable solvent, to a desired degree of viscosity, impregnating the gasket and subsequently evaporating off substantially all of the solvent.

3. A method of liquid proofing a gasket, including the preliminary partial decomposition of a metallic fatty acid salt to a gummy consistency, the dissolving of the resinous residue in a mixture of carbon tetrachloride and benzol, to a desired degree of viscosity, impregnating the gasket and subsequently evaporating off substantially all of the solvent.

BENJAMIN J. VICTOR.